



US009683280B2

(12) **United States Patent**  
**Muralidharan et al.**

(10) **Patent No.:** **US 9,683,280 B2**  
(45) **Date of Patent:** **Jun. 20, 2017**

(54) **INTERMEDIATE STRENGTH ALLOYS FOR HIGH TEMPERATURE SERVICE IN LIQUID-SALT COOLED ENERGY SYSTEMS**

(71) Applicant: **UT-Battelle, LLC**, Oak Ridge, TN (US)

(72) Inventors: **Govindarajan Muralidharan**, Knoxville, TN (US); **Dane Francis Wilson**, Oak Ridge, TN (US); **David Eugene Holcomb**, Oak Ridge, TN (US)

(73) Assignee: **UT-BATTELLE, LLC**, Oak Ridge, TN (US)

(\*) Notice: Subject to any disclaimer, the term of this patent is extended or adjusted under 35 U.S.C. 154(b) by 0 days.

(21) Appl. No.: **14/152,215**

(22) Filed: **Jan. 10, 2014**

(65) **Prior Publication Data**

US 2015/0197832 A1 Jul. 16, 2015

(51) **Int. Cl.**

**C22C 19/05** (2006.01)

(52) **U.S. Cl.**

CPC ..... **C22C 19/057** (2013.01)

(58) **Field of Classification Search**

CPC ..... C22C 1/023; C22C 1/0433; C22C 19/00; C22C 19/03; C22C 19/05; C22C 19/051; C22C 19/057

See application file for complete search history.

(56) **References Cited**

U.S. PATENT DOCUMENTS

|               |         |                                   |
|---------------|---------|-----------------------------------|
| 2,684,299 A   | 7/1954  | Binder                            |
| 3,030,206 A   | 4/1962  | Buck, Jr.                         |
| 3,416,916 A   | 12/1968 | Herchenroeder                     |
| 3,444,058 A   | 5/1969  | Mellors                           |
| 3,576,622 A   | 4/1971  | McCoy                             |
| 3,785,877 A * | 1/1974  | Bailey ..... C22F 1/10<br>148/556 |
| 3,811,960 A   | 5/1974  | Perry et al.                      |
| 3,917,463 A   | 11/1975 | Doi et al.                        |
| 3,985,582 A   | 10/1976 | Bibring et al.                    |
| 4,102,394 A   | 7/1978  | Boots                             |
| 4,194,909 A   | 3/1980  | Ohmura et al.                     |
| 4,476,091 A   | 10/1984 | Klarstrom                         |
| 4,512,817 A   | 4/1985  | Duhl et al.                       |
| 4,652,315 A   | 3/1987  | Igarashi et al.                   |
| 4,740,354 A   | 4/1988  | Watanabe et al.                   |
| 4,765,956 A   | 8/1988  | Smith et al.                      |
| 4,818,486 A   | 4/1989  | Rothman et al.                    |
| 4,820,359 A   | 4/1989  | Bevilacqua et al.                 |
| 4,877,461 A   | 10/1989 | Smith et al.                      |
| 5,077,006 A   | 12/1991 | Culling                           |
| 5,167,732 A   | 12/1992 | Naik                              |
| 5,244,515 A   | 9/1993  | Miglin                            |
| 5,330,590 A   | 7/1994  | Raj                               |
| 5,529,642 A   | 6/1996  | Sugahara et al.                   |
| 5,567,383 A   | 10/1996 | Noda et al.                       |
| 5,585,566 A   | 12/1996 | Welles, II et al.                 |
| 5,660,938 A   | 8/1997  | Sato et al.                       |
| 5,718,867 A   | 2/1998  | Nazmy et al.                      |

|              |         |                     |
|--------------|---------|---------------------|
| 5,779,972 A  | 7/1998  | Noda et al.         |
| 5,788,783 A  | 8/1998  | Couto et al.        |
| 5,888,316 A  | 3/1999  | Erickson            |
| 5,916,382 A  | 6/1999  | Sato                |
| 5,951,789 A  | 9/1999  | Ueta et al.         |
| 6,099,668 A  | 8/2000  | Ueta et al.         |
| 6,224,824 B1 | 5/2001  | Zhang et al.        |
| 6,344,097 B1 | 2/2002  | Limoges et al.      |
| 6,372,181 B1 | 4/2002  | Fahrmann            |
| 6,610,154 B2 | 8/2003  | Limoges et al.      |
| 6,702,905 B1 | 3/2004  | Qiao                |
| 6,797,232 B2 | 9/2004  | Speidel et al.      |
| 6,905,559 B2 | 6/2005  | O'Hara et al.       |
| 6,908,518 B2 | 6/2005  | Bouse et al.        |
| 7,011,721 B2 | 3/2006  | Harris et al.       |
| 7,038,585 B2 | 5/2006  | Hall et al.         |
| 7,042,365 B1 | 5/2006  | Diaz-Lopez et al.   |
| 7,089,902 B2 | 8/2006  | Sato et al.         |
| 7,160,400 B2 | 1/2007  | Magoshi et al.      |
| 7,450,023 B2 | 11/2008 | Muralidharan et al. |
| 7,507,306 B2 | 3/2009  | Chen et al.         |

(Continued)

FOREIGN PATENT DOCUMENTS

|    |         |         |
|----|---------|---------|
| CA | 706339  | 3/1965  |
| CA | 1215255 | 12/1986 |

(Continued)

OTHER PUBLICATIONS

Bruemmer, Stephen M. and Gary S. Was, Microstructural and Microchemical Mechanisms Controlling Intergranular Stress Corrosion Cracking in Light-Water-Reactor Systems, Journal of Nuclear Materials, 1994, pp. 348-363, , vol. 216.

Weitzel, P.S., Steam Generator for Advanced Ultra-Supercritical Power Plants 700 to 760C, Technical Paper, 2011, pp. 1-12.

Khan, T., The Development and Characterization of a High Performance Experimental Single Crystal Superalloy, pp. 145-155.

Freche, J.C., et al., Application of Powder Metallurgy to an Advanced-Temperature Nickel-Base Alloy, NASA-TN D-6560, pp. 1-22.

(Continued)

Primary Examiner — Roy King

Assistant Examiner — Jophy S Koshy

(74) Attorney, Agent, or Firm — Fox Rothschild LLP

(57) **ABSTRACT**

An alloy consists essentially of, in terms of weight percent: 6 to 8.5 Cr, 5.5 to 13.5 Mo, 0.4 to 7.5 W, 1 to 2 Ti, 0.7 to 0.85 Mn, 0.05 to 0.3 Al, up to 0.1 Co, 0.08 to 0.5 C, 1 to 5 Ta, 1 to 4 Nab, 1 to 3 Hf, balance Ni. The alloy is characterized by, at 850° C., a yield strength of at least 36 Ksi, a tensile strength of at least 40 Ksi, a creep rupture life at 12 Ksi of at least 72.1 hours, and a corrosion rate, expressed in weight loss [g/(cm<sup>2</sup>sec)]×10<sup>-11</sup> during a 1000 hour immersion in liquid FLiNaK at 850° C., in the range of 8 to 25.

(56)

## References Cited

## U.S. PATENT DOCUMENTS

|                 |         |                     |
|-----------------|---------|---------------------|
| 7,824,606 B2    | 11/2010 | Heazle              |
| 7,825,819 B2    | 11/2010 | Muralidharan et al. |
| 8,147,749 B2    | 4/2012  | Reynolds            |
| 8,313,591 B2    | 11/2012 | Hirata et al.       |
| 2003/0190906 A1 | 10/2003 | Winick              |
| 2004/0174260 A1 | 9/2004  | Wagner              |
| 2005/0053513 A1 | 3/2005  | Pike                |
| 2007/0152815 A1 | 7/2007  | Meyers et al.       |
| 2007/0152824 A1 | 7/2007  | Waterhouse et al.   |
| 2007/0152826 A1 | 7/2007  | August et al.       |
| 2007/0284018 A1 | 12/2007 | Hamano              |
| 2008/0001115 A1 | 1/2008  | Qiao et al.         |
| 2008/0126383 A1 | 5/2008  | Perrin              |
| 2009/0044884 A1 | 2/2009  | Toschi et al.       |
| 2009/0081073 A1 | 3/2009  | Barbosa et al.      |
| 2009/0081074 A1 | 3/2009  | Barbosa et al.      |
| 2009/0087338 A1 | 4/2009  | Mitchell et al.     |
| 2009/0194266 A1 | 8/2009  | Conrad et al.       |
| 2010/0008790 A1 | 1/2010  | Reynolds            |
| 2010/0116383 A1 | 5/2010  | Cloue et al.        |
| 2010/0303666 A1 | 12/2010 | Bain et al.         |
| 2010/0303669 A1 | 12/2010 | Pankiw et al.       |
| 2011/0236247 A1 | 9/2011  | Osaki et al.        |
| 2011/0272070 A1 | 11/2011 | Jakobi et al.       |
| 2012/0279351 A1 | 11/2012 | Gu et al.           |
| 2014/0271338 A1 | 9/2014  | Holcomb et al.      |

## FOREIGN PATENT DOCUMENTS

|    |            |           |
|----|------------|-----------|
| CA | 2688507    | 6/2011    |
| CA | 2688647    | 6/2011    |
| CN | 100410404  | 8/2008    |
| CN | 202883034  | 4/2013    |
| EP | 1647609    | 4/2006    |
| GB | 734210     | 7/1955    |
| GB | 943141 A   | * 11/1963 |
| JP | 5684445    | 7/1981    |
| JP | 07109539   | 4/1995    |
| JP | 2012219339 | 11/2012   |
| RU | 2479658    | 4/2013    |
| WO | 9206223    | 4/1992    |
| WO | 2008005241 | 1/2008    |
| WO | 2009145708 | 12/2009   |
| WO | 2013080684 | 6/2013    |

## OTHER PUBLICATIONS

- Ignatiev et al.: "Alloys compatibility in molten salt fluorides: Kurchatov Institute related experience", Journal of Nuclear Materials, 441 (2013), 592-603.
- Kondo et al.: "Corrosion characteristics of reduced activation ferritic steel, JLF-1 (8.92Cr-2W) in molten salts Flibe and Flinak, Fusion Engineering and Design", 84 (2009) 1081-1085.
- Kondo et al.: "High Performance Corrosion Resistance of Nickel-Based Alloys in Molten Salt FLiBe", Fusion Science and Technology, 56, Jul. 2009, 190-194.
- Delpach et al.: "MSFR: Material Issues and the Effect of Chemistry Control", GIF Symposium, Paris France, Sep. 9-10, 2009.

Liu et al.: "Investigation on corrosion behavior of Ni-based alloys in molten fluoride salt using synchrotron radiation techniques", Journal of Nuclear Materials, 440 (2013) 124-128.

Glazoff et al.: "Computational Thermodynamic Modeling of Hot Corrosion of Alloys Haynes 242 and HastelloyTM N For Molten Salt Service in Advanced High Temperature Reactors", Journal of Nuclear Energy Science & Power Generation Technology, 3(3), 2014.

Materials Compatibility for High Temperature Liquid Cooled Reactor Systems (RC-1) [https://neup.inl.gov/SiteAssets/FY\\_2017\\_Documents/FY17\\_CINR\\_DRAFT\\_WORKSCOPES.pdf](https://neup.inl.gov/SiteAssets/FY_2017_Documents/FY17_CINR_DRAFT_WORKSCOPES.pdf).

Zheng et al.: "Corrosion of 316L Stainless Steel and Hastelloy N Superalloy in Molten Eutectic LiF—NaF—KF Salt and Interaction with Graphite", Nuclear Technology, 188(2), 2014, p. 192.

Zheng et al.: "Corrosion of 316 Stainless Steel in High Temperature Molten Li<sub>2</sub>BeF<sub>4</sub> (FLiBe) Salt", Journal of Nuclear Materials, vol. 416, 2015, p. 143.

Olson et al.: Impact of Corrosion Test Container Material in Molten Fluorides, Journal of Solar Energy Engineering, v. 137(6), 061007, 2015.

Zheng et al.: "High Temperature Corrosion of Hastelloy N in Molten Li<sub>2</sub>BeF<sub>4</sub> (FLiBe) Salt", Corrosion, 71/10, 2015, p. 1257.

Barner, J.H. Von et al., "Vibrational Spectra of Fluoro and Oxofluoro Complexes of Nb(V) and Ta(V)", Materials Science Forum vols. 73-75 (1991) pp. 279-284 © (1991) Trans Tech Publications, Switzerland doi:10.4028/www.scientific.net/MSF.73-75.279.

Devan, Jackson H., "Effect of Alloying Additions on Corrosion Behaviour of Nickel-Molybdenum Alloys in Fused Fluoride Mixtures", ORNL-TM-2021, vol. I, J. H. DeVan; Oak Ridge National Laboratory Central Research Library Document Collection (May 1969).

Misra, Ajay K. et al., "Fluoride Salts and Container Materials for Thermal Energy Storage Applications in the Temperature Range 973 to 1400 K", 22nd Intersociety Energy Conversion Engineering Conference cosponsored by the AIAA, ANS, ASME, SAE, IEEE, ACS, and AIChE Philadelphia, Pennsylvania, Aug. 10-14, 1987. Department of Metallurgy and Materials Science, Case Western Reserve University , Cleve.

Polyakova, L.P. et al., "Electrochemical Study of Tantalum in Fluoride and Oxofluoride Melts", J. Electrochem. Soc., vol. 141, No. 11, Nov. 1994 The Electrochemical Society Inc., pp. 2982-2988.

Singh, Raj P. , "Processing of Ta<sub>2</sub>O<sub>5</sub> Powders for Electronic Applications", Journal of Electronic Materials, vol. 30, No. 12, 2001, pp. 1584-1594.

Yoder, Graydon L. et al., "An experimental test facility to support development of the fluoride-salt-cooled high-temperature reactor", Annals of Nuclear Energy 64 (2014) 511-517.

"Advanced Sensor System for Energy Infrastructure Assurance", Jan. 2004, Office of Energy Assurance, U.S Department of Energy, 2 pages.

ASM International, Materials Park, Ohio, Properties and Selection: Nonferrous Alloys and Special Purpose Materials: Nickel and Nickel Alloys, Oct. 1990, vol. 2, pp. 428-445.

\* cited by examiner



Fig. 1

**Fig. 2**



Fig. 3



Fig. 4



Fig. 5



Fig. 6



Fig. 7



Fig. 8



Fig. 9



Fig. 10



Fig. 11



Fig. 12



Fig. 13



Fig. 14

## INTERMEDIATE STRENGTH ALLOYS FOR HIGH TEMPERATURE SERVICE IN LIQUID-SALT COOLED ENERGY SYSTEMS

### STATEMENT REGARDING FEDERALLY SPONSORED RESEARCH

The United States Government has rights in this invention pursuant to contract no. DE-AC05-00OR22725 between the United States Department of Energy and UT-Battelle, LLC.

### CROSS-REFERENCE TO RELATED APPLICATIONS

This patent application is related to U.S. patent application Ser. No. 13/834,985 entitled "High Strength Alloys for High Temperature Service in Liquid-Salt Cooled Energy Systems" filed on Mar. 15, 2013, the entire disclosure of which is incorporated herein by reference. Moreover, this patent application is related to U.S. patent application Ser. No. 13/958,672 entitled "Creep-Resistant, Cobalt-Containing Alloys for High Temperature, Liquid-Salt Heat Exchanger Systems" filed on Aug. 5, 2013, the entire disclosure of which is incorporated herein by reference. Moreover, this patent application is related to U.S. patent application Ser. No. 13/962,197 entitled "Creep-Resistant, Cobalt-Free Alloys for High Temperature, Liquid-Salt Heat Exchanger Systems" filed on Aug. 8, 2013, the entire disclosure of which is incorporated herein by reference.

### BACKGROUND OF THE INVENTION

An ever-increasing demand for higher system thermal efficiency has necessitated the operation of power generation cycles and heat conversion systems for chemical processes at progressively higher temperatures. As system operating temperatures are increased, fewer materials with acceptable mechanical properties and environmental compatibility are known. This dearth of materials is particularly acute in applications at temperatures above 700° C. especially when accompanied by significant stress levels. Liquid fluoride salts are favored as heat transfer media at these high temperatures because of their high thermal capacity and low vapor pressure. There is, therefore, a need for fluoride salt compatible structural alloys for high-temperature heat transfer applications in order to enable increased thermal efficiency of energy conversion and transport systems thereby reducing system costs as well as reducing the waste heat rejected to the environment.

Fluoride salt cooled High temperature Reactors (FHRs) potentially have attractive performance and safety attributes. Defining features of FHRs include coated particle fuel, low-pressure fluoride salt cooling, and high-temperature heat production. The FHR heat transfer technology base is derived primarily from earlier molten salt reactors and their coated particle fuel is similar to that developed for high-temperature helium-cooled reactors. The excellent heat transfer characteristics of liquid fluoride salts enable full passive safety, at almost any power scale, thereby enabling large power output reactors with less massive piping and containment structures, and consequent economies of scale. FHRs potentially have improved economics, increased safety margins, and lower water usage characteristics than conventional water-cooled reactors.

The fuel and coolants for FHRs are suitable for operation at temperatures well in excess of the upper temperature limits of available structural alloys. A limiting factor in

achieving the highest possible FHR core outlet temperatures, and thus thermal efficiency, is the availability of structural alloys having sufficient creep strength at the required temperatures combined with suitable fluoride salt chemical compatibility as well as ease of fabrication and joining. Hastelloy® N (trademark owned by Haynes International, Inc.) (also known as Alloy N and INOR-8), developed at Oak Ridge National laboratory (ORNL) in the 1950s and 1960s, is currently a leading candidate FHR structural alloy for operations below 700° C. Hastelloy® N is limited to use in low stress applications to a maximum temperature of about 704° C. due to insufficient creep strength at higher temperatures, is limited to use in high stress applications such as steam generator tubes to about 600° C. due to insufficient creep strength at higher temperatures, is not fully qualified to current code requirements for high temperature reactors, and is challenging to fabricate due to its work hardening characteristics. There is therefore a need for corrosion-resistant nickel-based structural alloys designed to possess good creep resistance in liquid fluorides at higher temperatures in order to provide substantial improvements in FHR economics and performance. Calculations reveal that a net thermal efficiency of greater than 50% (as compared to about 33% net thermal efficiency of existing reactors) would be likely for FHRs using a high temperature structural alloy with concurrent reductions in capital costs, waste generation, fissile material requirements, and cooling water usage.

Other applications for these alloys include concentrated solar power (CSP), and processing equipment for fluoride environments. Molten-salt power towers are envisioned as operating in excess of 650° C. to achieve efficiency and cost targets. Temperatures of up to 700° C. are anticipated with the use of commercial supercritical steam turbines, up to 800° C. with the use of supercritical CO<sub>2</sub> Brayton cycle system, and even higher temperatures using open air Brayton cycle systems. Molten salts allow for the storage of solar energy and thus, the decoupling of solar energy collection from electricity generation. At the higher temperatures, molten fluoride salts offer the advantages of high thermal capacity, high heat transfer, and low vapor pressure. The development of materials with acceptable mechanical and molten salt corrosion resistance will allow for achieving the desired efficiency and cost targets.

Development of a high temperature structural alloy tailored to the specific high temperature strength and liquid salt corrosion resistance needs of liquid fluoride salt cooled-energy systems (especially FHRs) is contemplated to be of critical importance to ensuring feasibility and performance thereof. Simultaneously achieving creep resistance and liquid fluoride salt resistance at higher temperatures is challenging because conventional additions of certain alloying elements for achieving improved creep resistance and resistance to oxidation in air are detrimental to liquid fluoride salt resistance.

In general, conventional Ni-based alloys are strengthened through a combination of solid solution strengthening and precipitation strengthening mechanisms with the latter needed to achieve higher strengths at higher temperatures. In one class of Ni-based superalloys, primary strengthening is obtained through the homogeneous precipitation of ordered, L1<sub>2</sub> structured, Ni<sub>3</sub>(Al,Ti,Nb)-based intermetallic precipitates that are coherently embedded in a solid solution face centered cubic (FCC) matrix. In another class of Ni-based alloys, creep resistance is achieved through the precipitation of fine carbides (M<sub>23</sub>C<sub>6</sub>, M<sub>7</sub>C<sub>3</sub>, M<sub>6</sub>C where M is primarily Cr with substitution of Mo, W, for example) and carboni-

trides (M(C, N) where M is primarily Nb, or Ti, for example) within the matrix, and larger carbides on grain boundaries to prevent grain boundary sliding. Moreover, high temperature oxidation resistance in these alloys is obtained through additions of Cr and Al. Existing data (shown in FIG. 1) on liquid fluoride salt resistance of Ni-based alloys show that alloys containing aluminum and substantial amounts of chromium have lower resistance to liquid fluoride salt. Commercial nickel-based alloys with high strengths typically contain significant amounts of Cr (greater than 15 wt. % Cr) making them unsuitable for use in contact with liquid fluoride salts. Compositions (in weight %) of several commercially produced Ni-based alloys are shown in Table 1.

Hastelloy® N is an alloy that was designed to balance resistance to liquid fluoride salt corrosion with good creep properties at temperatures up to 704° C. This alloy is a Ni—Mo alloy containing additional alloying elements with solid solution strengthening being the primary strengthening mechanism; Hastelloy® N does not have  $\gamma'$  precipitation strengthening. Its nominal composition is given as



where \* indicates maximum allowed content of the indicated elements. Hastelloy® N generally consists of the following elements to provide the corresponding benefits:

Chromium: Added to ensure good oxidation resistance but minimized to keep liquid fluoride salt corrosion within acceptable limits. Also provides solid solution strengthening. Too much addition results in excessive attack by liquid fluoride salts.

Molybdenum: Principal strengthening addition for solid solution strengthening, provides good resistance to liquid fluoride salt, and results in lower interdiffusion coefficients. Also is the primary constituent in  $M_6C$  carbides. Too much addition can result in the formation of undesirable, brittle intermetallic phases.

Iron: Minimizes cost of alloy. Provides solid solution strengthening. Too much addition can destabilize austenitic matrix and decrease resistance to liquid fluoride salt.

Manganese: Stabilizes the austenitic matrix phase. Provides solid solution strengthening.

Silicon: Assists in high temperature oxidation resistance, a maximum of 1% Si may be added.

Carbon, Nitrogen: Required for the formation of carbide and/or carbonitride phases that can act as grain boundary pinning agents to minimize grain growth and to provide resistance to grain boundary sliding. Fine precipitation of carbide and/or carbonitride phases can increase high temperature strength and creep resistance.

Copper: Stabilizes the austenitic matrix, provides solid solution strengthening.

Cobalt: Provides solid solution strengthening. Co should not be present in alloys exposed to high neutron fluxes or whose corrosion products are exposed to high neutron fluxes, since these are subject to activation.

Tungsten: Provides solid solution strengthening and decreases average interdiffusion coefficient. Too much W can result in the formation of brittle intermetallic phases that can be deleterious to processability.

Aluminum+Titanium are not desirable in Hastelloy® N, in order to minimize corrosion by liquid salt. Combined wt. % of Al+Ti is typically kept to less than 0.35.

FIG. 1 shows effects of alloying element additions on the depth of corrosion of Ni-alloys in 54.3LiF-41.0KF-

11.2NaF-2.5UF<sub>4</sub> (mole percent) in a thermal convention loop operated between 815 and 650° C. (smaller depth of corrosion is better).

FIG. 2 shows the equilibrium phase fractions in Hastelloy® N as a function of temperature. Note that solid solution strengthening and some carbide strengthening (through  $M_6C$ ) are the primary strengthening mechanisms active in Hastelloy® N. This limits the strength and creep resistance of Hastelloy® N at high temperatures and restricts its useful temperatures to less than about 704° C. Components such as power cycle heat exchangers need to withstand large pressure differences between salt on one side of the heat exchanger wall and a gaseous working fluid at higher pressures on the other side. Such components hence need materials with high temperature strength greater than that of Hastelloy® N along with good resistance to salt, and good oxidation resistance.

#### BRIEF SUMMARY OF THE INVENTION

In accordance with one aspect of the present invention, the foregoing and other objects are achieved by an alloy consisting essentially of, in terms of weight percent: 6 to 8.5 Cr, 5.5 to 13.5 Mo, 0.4 to 7.5 W, 1 to 2 Ti, 0.7 to 0.85 Mn, 0.05 to 0.3 Al, up to 0.1 Co, 0.08 to 0.5 C, 1 to 5 Ta, 1 to 4 Nb, 1 to 3 Hf, balance Ni. The alloy is characterized by, at 850° C., a yield strength of at least 36 ksi, a tensile strength of at least 40 ksi, a creep rupture life at 12 ksi of at least 72.1 hours, and a corrosion rate, expressed in weight loss [g/(cm<sup>2</sup>sec)] $\times 10^{-11}$  during a 1000 hour immersion in liquid FLiNaK at 850° C., in the range of 8 to 25.

#### BRIEF DESCRIPTION OF THE DRAWINGS

FIG. 1 is a combination table and bar graph showing effects of alloying element additions on the depth of corrosion of Ni-alloys in 54.3LiF-41.0KF-11.2NaF-2.5UF<sub>4</sub> (mole percent) in a thermal convention loop operated between 815 and 650° C.

FIG. 2 is a graph showing phase equilibria for a typical composition of Hastelloy® N as a function of temperature (nitrogen and boron are not included in the calculations).

FIG. 3 is a graph showing phase equilibria for Alloy 3 as a function of temperature (nitrogen and boron are not included in the calculations).

FIG. 4 is an expanded view of a portion of the graph shown in FIG. 3 to show details.

FIG. 5 is a graph showing phase equilibria for Alloy 4 as a function of temperature (nitrogen and boron are not included in the calculations).

FIG. 6 is an expanded view of a portion of the graph shown in FIG. 5 to show details.

FIG. 7 is a graph showing phase equilibria for Alloy 5 as a function of temperature (nitrogen and boron are not included in the calculations).

FIG. 8 is an expanded view of a portion of the graph shown in FIG. 7 to show details.

FIG. 9 is a graph showing phase equilibria for Alloy 20 as a function of temperature (nitrogen and boron are not included in the calculations).

FIG. 10 is an expanded view of a portion of the graph shown in FIG. 9 to show details.

FIG. 11 is a graph showing phase equilibria for Alloy 22 as a function of temperature (nitrogen and boron are not included in the calculations).

FIG. 12 is an expanded view of a portion of the graph shown in FIG. 11 to show details.

FIG. 13 is a graph showing phase equilibria for Alloy 24 as a function of temperature (nitrogen and boron are not included in the calculations).

FIG. 14 is an expanded view of a portion of the graph shown in FIG. 13 to show details.

For a better understanding of the present invention, together with other and further objects, advantages and capabilities thereof, reference is made to the following disclosure and appended claims in connection with the above-described drawings.

#### DETAILED DESCRIPTION OF THE INVENTION

New, essentially Fe-free, solid-solution-strengthened alloys having improved high temperature strength and creep resistance; general composition limits are shown in Table 2. The primary strengthening in the new alloys is achieved through the precipitation of carbides along with solid solution strengthening. Moreover, the new alloys exhibit an advantageously lower average interdiffusion coefficient in the matrix. The skilled artisan will recognize that a lower interdiffusion rate results in, at high temperatures, lower coarsening rate of carbides, improved creep properties, lower oxidation rate, and lower corrosion rate.

Computational design was used to ensure that formation of brittle intermetallic phases that form in the new alloys is very low or zero weight % in the operating temperature range of contemplated greatest interest (750 to 950° C.). In the alloys, small amounts of carbide formers such as Ti, Nb, Hf, and Ta have been added to form carbides and the carbon levels have been increased as compared to Hastelloy® N. Carbides such as, for example, M<sub>6</sub>C and MC, or a combination thereof are present in these alloys in addition to the M<sub>6</sub>C carbides that are formed in Hastelloy® N.

The precipitate strengthened alloys described herein provide the higher strength required for applications for which the solid solution strengthened alloys have insufficient strength, and also provide improved creep strength. One disadvantage with conventional carbide strengthened alloys is that the strength decreases with time at temperature due to the coarsening of the carbide precipitates. The rate of loss of strength is directly related to the rate of growth of precipitates, which increases with increase in temperature (which also results in an increase in interdiffusion coefficients). The addition of sufficient amount of Mo, W, and/or Ta to the alloys of the present invention ensures that the interdiffusion coefficient is kept as low as reasonably possible and the coarsening rates are low, thus retaining properties for an extended period of time.

Broadest constituent ranges for alloys of the present invention are set forth in Table 2. Some examples thereof are set forth in Table 3, with Hastelloy® N for comparison. It is contemplated that alloys of the present invention may contain up to 5% Fe with concomitant reduction in some beneficial properties, such as creep resistance and oxidation resistance. Moreover, particularly in applications where the alloy is subject to nuclear radiation, cobalt may be eliminated to reduce activation with a small but concomitant reduction in strength and creep properties.

#### EXAMPLES

Alloys 3, 4, 5, 20, 22, and 24, shown in Table 3 were made using well known, conventional methods. Vacuum arc cast ingots were annealed at 1200° C. in an inert gas environment (vacuum can also be used). The ingots were then hot-rolled

into plates for mechanical testing. A solution annealing treatment was performed at 1150° C. for 1 hour. Thus, all the alloys can be cast, heat-treated, and mechanically processed into plates and sheets. The skilled artisan will recognize that other, conventional heat-treatment schedules can be used.

FIGS. 3-14 show the results from equilibrium calculations obtained from the computational thermodynamics software JMatPro v 6.2. Actual compositions were used for all the calculations.

Table 4 shows equilibrium wt. % of phases present in alloys at 850° C. It is essential that an alloy have M<sub>6</sub>C type carbides and at least one of MC type carbides and Ni<sub>5</sub>M type precipitates for optimum creep resistance. Small, finely dispersed carbides produced by heat-treatment improve creep resistance and are preferred over large carbides formed during solidification. Total precipitate phases must be present in a range of 4.0 to 10 wt. %. M<sub>6</sub>C type carbides must be present in a range of 1 to 8 wt. %. MC type carbides can be present in a range of up to 3.5 wt. %. Ni<sub>5</sub>M type precipitates can be present in a range of up to 3 wt. %. It is contemplated that more than 3 wt. % Ni<sub>5</sub>M type precipitates may be potentially deleterious to mechanical properties.

Yield and tensile strengths have been measured at 850° C. and compared with the baseline properties of Hastelloy® N and are shown in Table 5. Note that the yield strengths of the new alloys at 850° C. in the solution annealed condition are 2.5-26% better than that of Hastelloy® N. Typical yield strengths of alloys of the present invention are contemplated to be at least 36 ksi, preferably at least 40 ksi. Typical tensile strengths of alloys of the present invention are contemplated to be at least 40 ksi, preferably at least 50 ksi.

Creep rupture life has been measured in the solution annealed condition at 850° C. at a stress level of 12 ksi with the new alloys showing improvements in rupture lives of about 1812% to 4774%, as shown in Table 6. Creep rupture lives of alloys of the present invention are contemplated to be at least 72 hours, preferably at least 100 hours.

Resistances to liquid salt corrosion were measured by placing the alloy specimens of measured dimensions and weight in sealed molybdenum capsules in contact with a fixed amount of FLiNaK, a liquid salt heat exchange medium. The molybdenum capsules were enclosed in outer capsule to minimize high temperature air oxidation and heated in a furnace at 850° C. for 1,000 hours. After exposure, the capsules were opened and the specimens cleaned, weighed and their dimension measured. Corrosion resistance to liquid fluoride salt was evaluated based on normalized weight change and metallography and scanning electron microscopy. Results presented in Table 7 demonstrate that these alloys all have corrosion rates slightly higher than that of Hastelloy® N in these isothermal tests but with significantly improved mechanical properties. Thus a balance has been struck between improved mechanical properties and resistance to attack by liquid fluoride salt. Note that the aluminum and chromium has been kept at minimum required levels without adversely affecting the oxidation resistance and the salt resistance of these alloys. Typical corrosion rates of alloys of the present invention, expressed in weight loss [g/(cm<sup>2</sup>sec)] $\times 10^{-11}$  during a 1000 hour immersion in liquid FLiNaK at 850° C., are contemplated to be in the range of about 8 to about 25. Thus a balance has been struck between improved mechanical properties and resistance to attack by liquid fluoride salt.

Table 8 shows the relationship between the susceptibility to corrosion of the alloys shown by liquid fluoride salts, specifically FLiNaK with the Mo Equivalent, defined as

# US 9,683,280 B2

7

$$\text{Mo Equivalent} = \% \text{ Mo} + 1.15 \times \frac{183.84 \text{ (Atomic Weight of W)}}{95.95 \text{ (Atomic Weight of Mo)}} \times \% \text{ W}$$

where % refers to atomic percent of the element present in the alloy. 183.84 is the atomic wt. of W 95.95 is the atomic wt. of Mo. It has been observed that for these alloys the Mo Equivalent should be in the range of 5 to 12 for good resistance to liquid fluoride salts, specifically FLiNaK.

Table 8 shows the corrosion susceptibility index which quantifies the susceptibility to corrosion of the alloys shown in Table 3 by liquid fluoride salts, specifically FLiNaK. For this purpose, we define the corrosion susceptibility index as

$$CSI = \frac{\% \text{ Al} + \% \text{ Cr} + \% \text{ Ti} + \% \text{ Nb} + \% \text{ Hf} + \% \text{ Ta}}{\% \text{ Ni} + \% \text{ Fe} + \% \text{ Co} + \% \text{ Mn} + \% \text{ Mo} + \% \text{ W} + \% \text{ Re} + \% \text{ Ru}}$$

where % refers to atomic percent of the element present in the alloy. It has been observed that for these alloys, CSI should be no less than than about 0.1 and no greater than about 0.2 in addition to maintaining the elements in the preferred ranges. This results in the optimum combination of mechanical properties (high temperature strength and creep resistance) and resistance to fluoride salts.

10

Tables 1-8 follow.

While there has been shown and described what are at present considered to be examples of the invention, it will be obvious to those skilled in the art that various changes and modifications can be prepared therein without departing from the scope of the inventions defined by the appended claims.

TABLE 1

| Alloy       | Compositions of several commercial Ni-based alloys (in weight %). |      |      |      |      |      |      |      |      |      |     |      |      |      |      |
|-------------|-------------------------------------------------------------------|------|------|------|------|------|------|------|------|------|-----|------|------|------|------|
|             | C                                                                 | Si   | Mn   | Al   | Co   | Cr   | Cu   | Fe   | Mo   | Nb   | Ni  | Ta   | Ti   | W    | Zr   |
| X750        | 0.03                                                              | 0.09 | 0.08 | 0.68 | 0.04 | 15.7 | 0.08 | 8.03 | —    | 0.86 | Bal | 0.01 | 2.56 | —    | —    |
| Nimonic 80A | 0.08                                                              | 0.1  | 0.06 | 1.44 | 0.05 | 19.6 | 0.03 | 0.53 | —    | —    | Bal | —    | 2.53 | —    | —    |
| IN 751      | 0.03                                                              | 0.09 | 0.08 | 1.2  | 0.04 | 15.7 | 0.08 | 8.03 | —    | 0.86 | Bal | 0.01 | 2.56 | —    | —    |
| Nimonic 90  | 0.07                                                              | 0.18 | 0.07 | 1.4  | 16.1 | 19.4 | 0.04 | 0.51 | 0.09 | 0.02 | Bal | —    | 2.4  | —    | 0.07 |
| Waspaloy    | 0.03                                                              | 0.03 | 0.03 | 1.28 | 12.5 | 19.3 | 0.02 | 1.56 | 4.2  | —    | Bal | —    | 2.97 | —    | 0.05 |
| Rene 41     | 0.06                                                              | 0.01 | 0.01 | 1.6  | 10.6 | 18.4 | 0.01 | 0.2  | 9.9  | —    | Bal | —    | 3.2  | —    | —    |
| Udimet 520  | 0.04                                                              | 0.05 | 0.01 | 2.0  | 11.7 | 18.6 | 0.01 | 0.59 | 6.35 | —    | Bal | —    | 3.0  | —    | —    |
| Udimet 720  | 0.01                                                              | 0.01 | 0.01 | 2.5  | 14.8 | 15.9 | 0.01 | 0.12 | 3.0  | 0.01 | Bal | —    | 5.14 | 1.23 | 0.03 |
| Alloy 617   | 0.07                                                              | 0    | 0    | 1.2  | 12.5 | 22   | 0    | 1    | 9    | 0    | 54  | 0    | 0.3  | 0    | 0    |

TABLE 2

| 40 | Compositions of new alloys (analyzed compositions in wt. %) |               |               |
|----|-------------------------------------------------------------|---------------|---------------|
|    | Element                                                     | Minimum wt. % | Maximum wt. % |
| 45 | Cr                                                          | 6             | 8.5           |
|    | Mo                                                          | 5.5           | 13.5          |
|    | W                                                           | 0.4           | 7.5           |
|    | Ti                                                          | 1             | 2             |
|    | Mn                                                          | 0.7           | 0.85          |
|    | Al                                                          | 0.05          | 0.3           |
|    | Co                                                          | <0.005        | 0.1           |
|    | C                                                           | 0.08          | 0.5           |
|    | Ta                                                          | 1             | 5             |
|    | Nb                                                          | 1             | 4             |
|    | Hf                                                          | 1             | 3             |
|    | Fe                                                          | Essentially 0 |               |
| 50 | Ni                                                          | Balance       |               |

TABLE 3

| Alloy          | Compositions of new alloys compared to Hastelloy ® N (analyzed compositions in wt. %) |    |      |        |      |      |       |      |
|----------------|---------------------------------------------------------------------------------------|----|------|--------|------|------|-------|------|
|                | Ni                                                                                    | Fe | Al   | Co     | Cr   | Mn   | Mo    | Ti   |
| Hastelloy ® N* | 68.7                                                                                  | 5  |      | 0.2    | 7    | 0.8  | 16    | 0    |
| Alloy 3        | 73.87                                                                                 | 0  | 0.1  | 0.04   | 6.9  | 0.77 | 12.91 | 1.18 |
| Alloy 4        | 74.02                                                                                 | 0  | 0.1  | 0.0298 | 6.88 | 0.78 | 12.93 | 1.19 |
| Alloy 5        | 78.85                                                                                 | 0  | 0.09 | 0.02   | 6.7  | 0.79 | 8.17  | 1.18 |

TABLE 3-continued

| Compositions of new alloys compared to Hastelloy® N (analyzed compositions in wt. %) |      |      |      |      |      |      |        |       |
|--------------------------------------------------------------------------------------|------|------|------|------|------|------|--------|-------|
| Alloy                                                                                | Nb   | Hf   | Ta   | W    | C    | B**  | N**    | Total |
| Hastelloy® N*                                                                        | —    | 0    | 0    | 0.5  | 0.08 | 0.01 | —      | 100   |
| Alloy 3                                                                              | 1.06 | 1.16 | 1.19 | 0.59 | 0.23 | 0    | 0.0005 | 100   |
| Alloy 4                                                                              | 1.06 | 1.13 | 1.18 | 0.6  | 0.1  | 0    | 0.0002 | 100   |
| Alloy 5                                                                              | 1.09 | 1.16 | 1.18 | 0.52 | 0.25 | 0    | 0.0002 | 100   |
| Alloy 20                                                                             | 1.17 | 2.77 | 1.22 | 5.67 | 0.21 | 0    | 0.0005 | 100   |
| Alloy 22                                                                             | 3.76 | 1.15 | 1.2  | 6.99 | 0.19 | 0    | 0.0012 | 100   |
| Alloy 24                                                                             | 1.15 | 1.13 | 4.82 | 6.88 | 0.22 | 0    | 0.0037 | 100   |

\*Hastelloy® N also contains 1 Si, 0.35 Cu, 0.5 max of Al + Ti

\*\*Boron and Nitrogen are not included in the equilibrium calculations

TABLE 4

| Equilibrium wt. % of Phases Present in Alloys at 850° C. |                |                           |                       |                |                            |                          |
|----------------------------------------------------------|----------------|---------------------------|-----------------------|----------------|----------------------------|--------------------------|
| Alloy                                                    | Wt. % $\gamma$ | Wt. % $M_6C$ Precipitates | Wt. % MC Precipitates | Total Carbides | Wt. % $Ni_5M$ Precipitates | Total Precipitate Phases |
| Hastelloy® N                                             | 98.77          | 1.23                      | 0                     | 1.23           | 0                          | 1.23                     |
| Alloy 3                                                  | 90.68          | 7.54                      | 0.66                  | 8.20           | 1.12                       | 9.22                     |
| Alloy 4                                                  | 93.37          | 4.0                       | 0                     | 4.0            | 2.63                       | 6.63                     |
| Alloy 5                                                  | 92.83          | 5.78                      | 1.39                  | 7.17           | 0                          | 7.17                     |
| Alloy 20                                                 | 95.91          | 1.11                      | 2.98                  | 4.09           | 0                          | 4.09                     |
| Alloy 22                                                 | 95.93          | 2.31                      | 1.76                  | 4.07           | 0                          | 4.07                     |
| Alloy 24                                                 | 93.89          | 4.52                      | 1.59                  | 6.11           | 0                          | 6.11                     |

TABLE 5

| Yield and Tensile Strengths of Alloys at 850° C. and Improvement in Yield Strength over the baseline alloy. |                |                  |                                 |
|-------------------------------------------------------------------------------------------------------------|----------------|------------------|---------------------------------|
| Alloy                                                                                                       | Yield Strength | Tensile strength | % Improvement in Yield Strength |
| Hastelloy® N                                                                                                | 35.29          | 45.70            | 0                               |
| Alloy 3                                                                                                     | 41.67          | 49.93            | 18.1                            |
| Alloy 4                                                                                                     | 37.18          | 50.93            | 5.4                             |
| Alloy 5                                                                                                     | 36.18          | 40.30            | 2.5                             |
| Alloy 20                                                                                                    | 41.93          | 53.27            | 18.8                            |
| Alloy 22                                                                                                    | 44.35          | 57.27            | 25.7                            |
| Alloy 24                                                                                                    | 44.35          | 55.27            | 25.7                            |

TABLE 6

| Creep rupture lives of alloys at 850° C., at a stress of 12 ksi and improvement over the baseline alloy. |                              |                                     |
|----------------------------------------------------------------------------------------------------------|------------------------------|-------------------------------------|
| Alloy                                                                                                    | Creep Rupture Life           | % Improvement in creep rupture life |
| Hastelloy® N                                                                                             | 3.77<br>(average of 3 tests) | 0                                   |
| Alloy 3                                                                                                  | 183.7                        | 4773                                |
| Alloy 4                                                                                                  | 109                          | 2791                                |
| Alloy 5                                                                                                  | 72.1                         | 1812                                |
| Alloy 20                                                                                                 | 116                          | 2977                                |

TABLE 6-continued

| Creep rupture lives of alloys at 850° C., at a stress of 12 ksi and improvement over the baseline alloy. |                    |                                     |
|----------------------------------------------------------------------------------------------------------|--------------------|-------------------------------------|
| Alloy                                                                                                    | Creep Rupture Life | % Improvement in creep rupture life |
| Alloy 22                                                                                                 | 128.8              | 3316                                |
| Alloy 24                                                                                                 | 138.2              | 3566                                |

TABLE 7

| Corrosion Rate (Weight Loss) Measured During a 1000 hour immersion in liquid FLiNaK at 850° C. |                                        |  |
|------------------------------------------------------------------------------------------------|----------------------------------------|--|
| Alloy                                                                                          | Corrosion rate [g/(cm²sec)] $10^{-11}$ |  |
| Hastelloy® N                                                                                   | 1.21                                   |  |
| Alloy 3                                                                                        | 20.34                                  |  |
| Alloy 4                                                                                        | 21.87                                  |  |
| Alloy 5                                                                                        | 22.99                                  |  |
| Alloy 20                                                                                       | 11.28                                  |  |
| Alloy 22                                                                                       | 10.43                                  |  |
| Alloy 24                                                                                       | 16.06                                  |  |

TABLE 8

| Composition of alloys in at. % and the calculation of Mo Equivalent and Corrosion Susceptibility Index (CSI) |         |         |       |        |       |         |          |       |
|--------------------------------------------------------------------------------------------------------------|---------|---------|-------|--------|-------|---------|----------|-------|
| Alloy                                                                                                        | Ni      | Fe      | Al    | Co     | Cr    | Mn      | Mo       | Ti    |
| Hastelloy ® N*                                                                                               | 75.735  | 4.443   | 0     | 0.157  | 7.473 | 0.594   | 10.34    | 0     |
| Alloy 3                                                                                                      | 77.8959 | 0       | 0.229 | 0.0421 | 8.213 | 0.867   | 8.328    | 1.526 |
| Alloy 4                                                                                                      | 78.4595 | 0       | 0.231 | 0.0315 | 8.232 | 0.883   | 8.385    | 1.547 |
| Alloy 5                                                                                                      | 81.492  | 0       | 0.202 | 0.02   | 7.816 | 0.872   | 5.166    | 1.495 |
| Alloy 20                                                                                                     | 78.3326 | 0.01139 | 0.212 | 0.01   | 8.672 | 0.891   | 4.959    | 1.621 |
| Alloy 22                                                                                                     | 76.516  | 0       | 0.189 | 0.086  | 10.07 | 0.869   | 3.854    | 1.582 |
| Alloy 24                                                                                                     | 78.2414 | 0.01158 | 0.264 | 0.01   | 8.495 | 0.895   | 3.991    | 1.554 |
| Alloy                                                                                                        | Nb      | Hf      | Ta    | W      | C     | Mo Equ. | CSI      |       |
| Hastelloy ® N*                                                                                               | 0       | 0       | 0     | 0.02   | 0.154 | 10.38   | 0.081861 |       |
| Alloy 3                                                                                                      | 0.706   | 0.402   | 0.407 | 0.199  | 1.185 | 8.77    | 0.1315   |       |
| Alloy 4                                                                                                      | 0.71    | 0.394   | 0.406 | 0.203  | 0.518 | 8.83    | 0.1310   |       |
| Alloy 5                                                                                                      | 0.712   | 0.394   | 0.396 | 0.172  | 1.263 | 5.55    | 0.1256   |       |
| Alloy 20                                                                                                     | 0.801   | 0.987   | 0.429 | 1.962  | 1.112 | 9.28    | 0.1476   |       |
| Alloy 22                                                                                                     | 2.575   | 0.41    | 0.422 | 2.42   | 1.007 | 9.19    | 0.1821   |       |
| Alloy 24                                                                                                     | 0.801   | 0.409   | 1.723 | 2.42   | 1.185 | 9.32    | 0.1548   |       |

What is claimed is:

1. An alloy for use in components in contact with liquid fluorides, consisting essentially of, in terms of weight percent:

Cr: 6 to 8.5,  
Mo: 5.5 to 13.5,  
W: 0.4 to 7.5,  
Ti: 1 to 2,  
Mn: 0.7 to 0.85,  
Al: 0.05 to 0.3,  
Co: 0 to 0.1,  
C: 0.08 to 0.5,  
Ta: 1 to 5,  
Nb: 1 to 4,  
Hf: 1 to 3,  
Fe: ≤0.01,  
Ni: balance,  
with Al+Ti≤2.3 wt. %;

and said alloy being characterized by

i) at alloy temperatures of 850° C., a yield strength of at least 36 Ksi, a tensile strength of at least 40 Ksi, a creep rupture life at 12 Ksi of at least 72.1 hours, and a corrosion rate of  $8 \times 10^{-11}$  g/cm<sup>2</sup>s to  $25 \times 10^{-11}$  g/cm<sup>2</sup>s of weight loss during a 1000 hour immersion in liquid FLiNaK at 850° C.;  
ii) at alloy temperatures of 850° C., a matrix consisting of γ and 4.0 to 10 wt. % total precipitates, said total precipitates consisting of at least one M<sub>6</sub>C type carbide and at least one additional precipitate selected from the group consisting of MC type carbides and Ni<sub>5</sub>M type precipitates;  
iii) said alloy possessing an Mo Equivalent of no less than 5, wherein,

$$\text{Mo Equivalent} = \% \text{ Mo} + 1.15 \times \frac{183.84}{95.95} \times \% \text{ W}$$

and iv) said alloy having a corrosion susceptibility index, CSI, of no less than about 0.1 and no more than about 0.2, wherein

$$CSI = \frac{\% \text{ Al} + \% \text{ Cr} + \% \text{ Ti} + \% \text{ Nb} + \% \text{ Hf} + \% \text{ Ta}}{\% \text{ Ni} + \% \text{ Fe} + \% \text{ Co} + \% \text{ Mn} + \% \text{ Mo} + \% \text{ W} + \% \text{ Re} + \% \text{ Ru}}.$$

2. An alloy in accordance with claim 1 wherein the range of Cr is 6.7 to 8.3 weight percent.  
3. An alloy in accordance with claim 1 wherein the range of Mo is 5.81 to 12.93 weight percent.  
4. An alloy in accordance with claim 1 wherein the range of W is 0.52 to 6.99 weight percent.  
5. An alloy in accordance with claim 1 wherein the range of Ti is 1.15 to 1.22 weight percent.  
6. An alloy in accordance with claim 1 wherein the range of Mn is 0.75 to 0.79 weight percent.  
7. An alloy in accordance with claim 1 wherein the range of Al is 0.08 to 0.11 weight percent.  
8. An alloy in accordance with claim 1 wherein the range of Co is 0.01 to 0.08 weight percent.  
9. An alloy in accordance with claim 1 wherein the range of Ta is 1.18 to 4.82 weight percent.  
10. An alloy in accordance with claim 1 wherein the range of Nb is 1.06 to 3.76 weight percent.  
11. An alloy in accordance with claim 1 wherein the range of Hf is 1.13 to 2.77 weight percent.  
12. An alloy in accordance with claim 1 wherein the range of C is 0.1 to 0.25 weight percent.  
13. An alloy in accordance with claim 1 wherein said alloy is further characterized by 1 to 8 wt. % M<sub>6</sub>C type carbides.  
14. An alloy in accordance with claim 1 wherein said alloy is further characterized by up to 3.5 wt. % MC type carbides.  
15. An alloy in accordance with claim 1 wherein said alloy is further characterized by up to 3 wt. % Ni<sub>5</sub>M type precipitates.

\* \* \* \* \*